

## 1

3,238,044

## ONE-COMPONENT DIAZOTYPE MATERIAL

Hubertus Wilhelmus Henricus Maria Roncken and Andri-  
anus Marie Petrus Hectors, Venlo, Netherlands, assign-  
ors to Chemische Fabriek L. van der Grinten N.V.,  
Venlo, Netherlands, a corporation of Dutch law  
No Drawing. Filed Sept. 17, 1962, Ser. No. 224,237  
Claims priority, application Netherlands, Mar. 14, 1962,  
275,942

7 Claims. (Cl. 96—75)

The invention relates to one-component diazotype mate-  
rial.

In practice one-component diazotype materials which have been sensitized with 4-diazo-2-chloro-N,N-diethyl-  
aniline are used on a large scale. They are developed according to the so-called thin-layer method with weakly  
alkaline developing liquids which contain phloroglucinol,  
if desired together with resorcinol, and then yield copies with brown azo-dyestuff images that have high absorption  
for ultraviolet rays and are extremely suitable for use as  
intermediate originals if the support material is trans-  
lucent.

The brown colour of the azo-dyestuff of the copies on these diazotype materials, developed with weakly alkaline  
phloroglucinol developer, is not appreciated by all users of these materials. Many of them consider it too light.  
The copies sometimes show "bleeding" of the azo-dyestuff, in consequence of which the images are less sharp. This  
bleeding may be due to the dissolution of the diazo compound in the developing liquid during development, the  
azo-dyestuff formed from the dissolved diazo compound being deposited beyond the azo-dyestuff portions of the  
image on the surface of the copy. It may also be due to the azo-dyestuff formed in the azo-dyestuff portions  
being washed away with the developing liquid.

The bleeding occurs, for instance, if foam is formed in the developing liquid during the development of the copies. These diazotype materials are not suitable for development with weakly acid buffered phloroglucinol developers, because the diazo compound does not couple  
sufficiently actively. As is known, weakly acid buffered phloroglucinol developers have better keeping qualities than weakly alkaline phloroglucinol developers.

The South African Patent No. 3,627/60 describes one-component diazotype material which comprises a diazo film layer, sensitized with a diazo compound that couples more actively than 4-diazo-2-chloro-N,N-diethylaniline. This diazotype material can be developed with weakly acid liquids containing phloroglucinol and, if desired, resorcinol, which liquids have been buffered with a salt of a strong base and a dicarboxylic acid such as succinic acid, glutaric acid, adipic acid, and  $\beta$ -methyladipic acid.

The said South African patent describes, among other things, transparent diazotype material with a diazo film layer in which 4-diazo-2-chloro-N-methyl-N-cyclohexyl-  
aniline is present as diazo compound. This material is developed with a liquid which contains phloroglucinol and resorcinol as azo components and a mixture of sodium succinate, succinic acid, and sodium benzoate as buffer. The pH of this liquid is 6.6. After the application of the developing liquid the copy is dried while heating moderately. Upon development, copies are obtained with strong, dark violet-brown azo-dyestuff images on a clear transparent background. The azo-dyestuff has very good absorption for ultraviolet light and hardly bleaches upon prolonged or repeated exposure to this light.

For the development of diazotype materials sensitized with 4-diazo-2-chloro - N - methyl - N - cyclohexylaniline, either in a film layer or not, with a weakly acid phloroglucinol developer, the use of the said special weakly acid buffered phloroglucinol developer is more or less required

## 2

and the copies have to be heated after the application of the developing liquid in order to ensure proper development. Nevertheless, the developing speed of these materials is often too slow for practical purposes (even when the said special developer is used) if their light-sensitive layer contains the diazo compound in the form of the zinc chloride double salt together with the stabilizer 1,3,6-naphthalene trisulphonic acid or a water-soluble salt thereof. The use of the zinc chloride double salt of the diazo compound together with this stabilizer is highly desirable, because these diazotype materials otherwise are not very durable.

When the zinc chloride double salt of the diazo compound is used, however, the material is developed much less satisfactorily according to the thin-layer method than when, for instance, the chloride or the two-basic sulphate is used.

Moreover 1,3,6-naphthalene trisulphonic acid retards the coupling activity of 4-diazo-2-chloro-N-methyl-N-  
cyclohexylaniline in a high degree. The degree of retardation is indeed dependent on the quantity of stabilizer that is added, but it is already considerable upon addition of the usual quantity desirable for good stabilization.

If with a weakly acid buffered phloroglucinol developer a proper development of copies on diazotype material sensitized with the zinc chloride double salt of 4-diazo-2-chloro-N-methyl-N-cyclohexylaniline containing a conventional quantity of 1,3,6-naphthalene trisulphonic acid is to be obtained, it is necessary to provide, for instance, for a relatively high temperature of the developing liquid, such as 30 to 35°C., or for thorough heating of the copy wetted with the developing liquid, or for the application of a thick layer of developing liquid, such as 12 g./m.<sup>2</sup>, on the surface of the copy, or for a large quantity of phloroglucinol in the developing liquid.

The retarded developing speed may have all sorts of harmful consequences. Thus the visual and the transmission contrast of a copy which has been exposed to daylight for some time, for instance, may be considerably lower than that of a freshly developed copy, because the diazo compound that has not been converted into azo-dyestuff during development bleaches gradually. Furthermore the copies which originally had a clear background are often found to show "fogging" in the background portions after a few minutes in consequence of the slowness with which the development proceeds in those portions in which after the imagewise exposure only a small amount of diazo compound is left. Consequently, the quality of the copies can only be judged some time after development, a circumstance which is naturally very inconvenient in practice. Moreover the copies often show "bleeding."

From Dutch patent specification 36,214 one-component diazo-type material is known which has been made light-sensitive with 4-diazo - 2,5 - dichloro-N-(2',6'-dichloro)-benzylaniline. This material is developed with a weakly alkaline phloroglucinol-containing liquid, but it is only slightly light-sensitive according to present-day standards. The diazo compound does not couple sufficiently actively for the development of the diazotype material sensitized with it, according to the thin-layer method with a weakly acid buffered phloroglucinol developer.

From FIAT Report 813, page 1349, the compound 4-diazo-2,5-dichloro-N-ethyl-N-benzylaniline is known. No statement is made about its properties and about those of diazotype material sensitized with it. From a test, however, it appeared that this diazo compound forms a precipitate with 1,3,6-naphthalene trisulphonic acid in the conventional aqueous sensitizing liquids, so that it is not possible to use this diazo compound for making diazotype paper containing this stabilizer in the usual way.

Paper with this diazo compound without this stabilizer has very poor keeping qualities.

Now it has been found that one-component diazotype material containing a diazo compound of the general formula



in which X is an anion, R<sub>1</sub> and R<sub>2</sub> are chlorine or bromine atoms, and the cyclohexyl group may be substituted by one or more methyl radicals, can be stabilized in the usual way with 1,3,6-naphthalene trisulphonic acid or a salt thereof, without the coupling activity of the diazo compound, in this case the developing speed of the diazotype material, decreasing in a degree that is inconvenient for practical purposes.

The diazotype material according to the invention is very light-sensitive and it can be developed with weakly acid buffered phloroglucinol-containing developing liquids to form dark, almost black azo-dyestuffs which have high absorption for actinic radiation, and with weakly alkaline phloroglucinol-containing developing liquids to form fine dark-brown azo-dyestuffs which also have high absorption for actinic radiation.

The azo-dyestuff images obtained with weakly acid buffered phloroglucinol developers do not, or in a much less degree, show the above-mentioned phenomena, which point to incomplete development. When diazotype material according to the invention is used, bleeding of the azo-dyestuff image occurs in a much less degree than when diazotype material sensitized with 4-diazo-2-chlorodiethylaniline or 4 - diazo - 2 - chloro - N-methyl-N-cyclohexylaniline is used.

The support of the diazotype material according to the invention may be opaque, such as paper, linen, lacquered paper, or translucent, such as tracing paper that may or may not be lacquered, tracing linen, cellulose acetate and polyester film. If the support surface is hydrophobic, the diazo compound is preferably applied in a hydrophilic film layer which covers the hydrophobic surface. If the support is transparent or at least translucent, the copies are very suitable as intermediate originals, irrespective of whether they are developed with a weakly acid or with a weakly alkaline phloroglucinol developer.

Very attractive material is one-component diazotype material according to the invention which comprises a transparent support, such as natural tracing paper, tracing linen, or polyester film that has been coated with a film layer formed from a hydrophilic colloid obtained by hydrolysis of an ester of the group formed by cellulose and polyvinyl esters, in which film layer the diazo compound is present along with 1,3,6-naphthalene trisulphonic acid or a water-soluble salt thereof.

This diazotype material has good keeping qualities, is developed practically completely within a short time with a weakly acid buffered phloroglucinol-containing developing liquid according to the thin-layer method, and yields sharp copies with strong dark azo-dyestuff images, which have high absorption for ultraviolet light. The azo-dyestuff images of the copies can be readily erased, for instance by scraping off the film layer with a blade.

The keeping qualities of diazotype material according to the invention in which the diazo compound is present in the form of the zinc chloride double salt along with 1,3,6-naphthalene trisulphonic acid or a water-soluble salt thereof in a hydrophilic film layer as described above are particularly good. Notwithstanding the use of the diazo compound in the form of the zinc chloride double salt, such diazotype material is developed sufficiently rapidly with the weakly acid buffered phloroglucinol-containing developing liquids.

Diazo compounds which are suitable for application in the diazotype material according to the invention are, for instance:

- 5 4-diazo-3,6-dichloro-N-methyl-N-cyclohexylaniline  
4-diazo-3,6-dibromo-N-methyl-N-cyclohexylaniline  
4-diazo-3-chloro-6-bromo-N-methyl-N-cyclohexylaniline  
4-diazo-3,6-dichloro-N-methyl-N-(methyl)cyclohexyl-aniline

10 They can be used separately, mixed together, or mixed with another diazo compound.

They can be prepared as follows: 4-nitro-2-chloroaniline is diazotized and the diazo group is replaced by a chlorine or bromine atom by sandmeyering. The nitro group of the product obtained is reduced to an amino group, which is acetylated with acetic anhydride. In the 3-chloro-4-(chloro or bromo)acetanilide thus produced a nitro group is then introduced and the acetylaminogroup is deacetylated by boiling with hydrochloric acid, after which the 4-(chloro or bromo)-5-chloro - 2 - nitroaniline thus obtained is converted with N-cyclohexylamine into 5-cyclohexylamino - 4 - (chloro or bromo)-2-nitroaniline, from which compound 4-nitro-2-(chloro or bromo)-5-(chloro or bromo)-N-methyl-N-cyclohexylaniline is then obtained by diazotization, sandmeyering to chloro or bromo, and methylation with formic acid formaldehyde. Finally the nitro group is reduced and the amino compound obtained is diazotized, so that 4-N-methyl-N-cyclohexylamino-3-(chloro or bromo)-6-(chloro or bromo)-diazobenzene is obtained, which can be made available in the form of a salt, such as the zinc chloride double salt, chloro stannate, or boro fluoride.

35 The diazotype material according to the invention may contain the auxiliary agents commonly used in one-component diazotype material, for instance acids such as citric acid, boric acid, tartaric acid, stabilizers such as 1,3,6-naphthalene trisulphonic acid and its water-soluble salts, reducing agents such as thiourea, metal salts such as aluminum sulphate, synthetic resin dispersions, silica dispersions, etc.

#### Example I

Sized natural tracing paper is sensitized with a liquid containing:

- 45 64 g. of 4-N-methyl-N-cyclohexylamino-3,6-dibromobenzene diazonium chloride, zinc chloride double salt  
5 g. of tartaric acid  
20 g. of 1,3,6-naphthalene trisulphonic acid sodium salt  
50 30 ml. of polyvinyl acetate dispersion Vinnapas H. 60  
from Wacker-Chemie G.m.b.H., Munich  
1000 ml. of water  
and dried.

The transparent diazotype paper thus prepared is very light-sensitive and has good keeping qualities.

55 A sheet of the diazotype material is imagewise exposed underneath an ink tracing until underneath the blank portions of the tracing all the diazo compound has been bleached out, and then developed according to the so-called thin-layer method with a weakly acid liquid containing:

- 60 10 g. of thiourea  
6.5 g. of phloroglucinol  
4 g. of resorcinol  
65 2 g. of isopropynaphthalene sulphonic acid sodium salt  
14 g. of sodium formate  
22 g. of sodium benzoate  
47 g. of sodium citrate, 2 aq.  
1.2 g. of citric acid  
70 1000 ml. of water

The developing liquid has a pH of about 6.2.

The copy obtained shows a strong violet-black azo-dyestuff image on a clear background and is eminently suitable for use as an intermediate original for making fur-

ther copies. The azo-dyestuff image does not bleed upon development.

If instead of the above-mentioned diazo compound the zinc chloride double salt of 4-N-methyl-N-cyclohexylamino-3-chlorobenzene diazonium chloride had been used in an equivalent quantity, a less rapidly developing diazotype material of approximately the same light-sensitivity would have been obtained, which yields copies with somewhat lighter azo-dyestuff images, having good absorption for ultraviolet radiation, but showing some bleeding upon development.

Another sheet of the diazotype material is imagewise exposed as described above and then developed with a weakly alkaline liquid of the following composition:

30 g. of thiourea  
5.4 g. of phloroglucinol  
6.5 g. of resorcinol  
1 g. of hydroquinone monosulphonic acid potassium salt  
5 g. of sorbitol  
15 g. of sugar  
50 g. of potassium tetraborate, 5 aq.  
1.5 g. of isopropylnaphthalene sulphonate sodium salt  
1000 ml. of water

The developing liquid has a pH of about 9.5.

The copy obtained shows a strong, sharp, and fine dark-brown azo-dyestuff image, the azo-dyestuff of which has high absorption for ultraviolet radiation.

#### Example II

A cellulose acetate film layer of about 20 g./m., applied on natural tracing paper of about 80 g./m.<sup>2</sup>, is superficially hydrolysed to a depth of about 4 microns and, after washing with water to remove the chemicals used for the hydrolysis, is sensitized with a solution of:

65 g. of 4-N-methyl-N-cyclohexylamino-3,6-dichlorobenzene diazonium chloride, zinc chloride double salt  
2 g. of boric acid  
4 g. of tartaric acid  
20 g. of 1,3,6-naphthalene trisulphonic acid sodium salt  
250 ml. of ethanol (96%)  
750 ml. of water

and dried.

The diazotype material obtained is very light-sensitive and has excellent keeping qualities.

A sheet of the diazotype material is imagewise exposed as in Example I and developed with the weakly acid developing liquid mentioned in that example. The diazotype material has a markedly greater developing speed and yields markedly sharper and even darker-coloured azo-dyestuff images than corresponding diazotype material which contains an equivalent quantity of the zinc chloride double salt of 4-N-methyl-N-cyclohexylamino-3-chlorobenzene diazonium chloride.

Upon development with the weakly alkaline developing liquid described in Example I, the new diazotype material yields transparent copies with a strong dark-brown azo-dyestuff image, the azo-dyestuff of which has high absorption for ultraviolet radiation.

#### Example III

White base-paper of 80 g./m.<sup>2</sup> for the diazotype process is sensitized on one side with a solution of:

30 g. of 4-N-methyl-N-(methyl)cyclohexylamino-3,6-dichlorobenzene diazonium chloride, zinc chloride double salt  
5 g. of tartaric acid  
30 g. of 1,3,6-naphthalene trisulphonic acid sodium salt  
30 ml. of Vinnapas H. 60 in  
1000 ml. of water

and dried.

The diazotype paper obtained is very light-sensitive and has excellent keeping qualities.

A sheet of the diazotype paper is imagewise exposed as in Example I and then developed with a thin layer of the weakly acid developing liquid described in Example I. The copy shows a sharp and strong violet-black azo-dyestuff image on a clear white background.

If the new diazotype material is developed with the weakly alkaline developing liquid described in Example I, the azo-dyestuff image has a fine dark-brown shade.

A copy on a diazotype paper sensitized with a liquid of the same composition, but containing instead of the above-mentioned diazo compound an equivalent quantity of 4-N-methyl-N-cyclohexylamino-3-chlorobenzene diazonium chloride, zinc chloride double salt, if also developed with the weakly acid developing liquid, shows an incompletely developed, rather weak azo-dyestuff image, which moreover shows some bleeding of the lines.

#### Example IV

White paper of 150 g./m.<sup>2</sup>, provided on one side with a cellulose acetate film layer (approximately 50% by weight of combined acetic acid) of a thickness of about 10 microns, which has been fixed to the paper by means of an adhesive and which has been deacylated to a depth of about 4 microns to an average acetyl content, calculated as combined acetic acid, of approximately 20% by weight (which corresponds to an average number of acyl groups on the OH— groups of 0.7), is impregnated for 2.5 minutes on the deacylated side of the cellulose acetate layer with the following solution:

30 49 g. of 4-N-methyl-N-cyclohexylamino-3-chloro-6-bromobenzene diazonium chloride, zinc chloride double salt  
5 g. of tartaric acid  
35 20 g. of 1,3,6-naphthalene trisulphonic acid sodium salt  
250 ml. of ethanol (96%)  
750 ml. of water

and thus sensitized.

The excess of liquid is removed from the cellulose acetate surface and subsequently the material is dried. The diazotype material obtained is very light-sensitive and has good keeping qualities.

A sheet of the diazotype material is imagewise exposed as in Example I and developed with the weakly acid developing liquid described in that example. The copy obtained shows a very strong violet-black azo-dyestuff image, which did not bleed upon development. If instead of the weakly acid developer the weakly alkaline phloroglucinol developer described in Example I had been used, a copy with a very strong, fine dark-brown azo-dyestuff image would have been obtained.

If a similar sheet is sensitized in the same way with a solution of the same composition, but containing instead of the above-mentioned diazo compound an equivalent quantity of 4-N-methyl-N-cyclohexylamino-3-chlorobenzene diazonium chloride, zinc chloride double salt, a diazotype material is obtained which develops markedly less rapidly and yields copies with a dark red-brown azo-dyestuff image would have been obtained.

60 is effected with the weakly acid developer, and copies with a light-brown azo-dyestuff image if development is carried out with the weakly alkaline developer.

#### Example V

65 Tracing linen of the Red Bridge Sub./0/86 type from Red Bridge Book Cloth Company, Red Bridge, Ainsworth, Bolton, England, is coated by immersion with a layer of about 70 g./m.<sup>2</sup> of the following liquid:

70 100 g. of polystyrene copolymer Lutron X-820 from Monsanto Chemical Company, Plastics Division, Springfield 2, Massachusetts, U.S.A.  
30 g. of polyvinyl acetate Rhodopas H.V. 2 from Rhone-Poulenc, Paris, France  
50 ml. of ethyl acetate  
75 900 ml. of ethanol (96%)

After drying, a layer of about 80 g./m.<sup>2</sup> of the following liquid is applied on the hydrophobic adhesive layer thus formed:

40 g. of partially (about 53%) hydrolysed polyvinyl acetate Vinnapas U.W. 50 from Wacker-Chemie G.m.b.H., Munich 2, Germany

20 g. of Gelvatol 40-20, a partially hydrolysed polyvinyl acetate from Shawinigan Products Corp., New York 1, U.S.A.

5 g. of isopropylnaphthalene sulphonic acid sodium salt Aerosol OS from American Cyanamid Co., New York 20, U.S.A.

500 ml. of ethanol (96%)

500 ml. of water

After drying, a hydrophilic polyvinyl acetate layer of a thickness of about 4.5 microns is present on the adhesive layer.

Subsequently a sensitizing liquid is prepared as follows.

To a solution containing:

3.25 g. of 4-N-methyl-N-cyclohexylamino-2,5-dichloroaniline

3 ml. of hydrochloric acid (S. G. 1.19)

50 ml. of water of 0° C.

is added dropwise, with continuous stirring, while the solution is kept at a temperature of 2-5° C., such a quantity of a solution of:

30 g. of sodium nitrite in

100 ml. of water

that exactly all the amino compound is converted into the corresponding diazonium compound. To the diazonium chloride solution are then added

0.5 g. of tartaric acid

3 g. of naphthalene trisulphonic acid sodium salt

40 ml. of ethanol (96%) and

7 ml. of water

The hydrophilic polyvinyl acetate layer is impregnated with this sensitizing liquid.

The hydrophilic light-sensitive layer obtained after drying contains approximately 0.8 millimol of diazo compound per m.<sup>2</sup> of the sensitized surface.

A sheet of the transparent diazotype linen thus produced is imagewise exposed as in Example I and developed with the weakly acid developing liquid.

The copy obtained shows a dark violet-brown azo-dye-stuff image with good absorption for ultraviolet radiation. It is eminently suitable for use as an intermediate original for making further copies. The image on the copy can easily be removed (erased) locally, for instance by scraping off parts of the hydrophilic layer containing the azo-dye-stuff image.

A copy also having good absorption of the azo-dye-stuff image is obtained upon development with the weakly alkaline developing liquid described in Example I. In this case the azo-dye-stuff image has a brown shade.

If the hydrophilic polyvinyl acetate layer is impregnated with a sensitizing liquid prepared in the same way, but starting from 4-N-methyl-N-cyclohexylamino-3-chloroaniline, after the drying process a light-sensitive material is obtained which practically cannot be developed with the weakly acid developing liquid. A reasonable, though very slow, development is achieved if the quantity of 1,3,6-naphthalene trisulphonic acid sodium salt is reduced to one third of the original quantity.

Copies made on such material show a less strong dark-brown azo-dye-stuff image of a lighter shade, having good absorption for ultraviolet radiation.

We claim:

1. One-component diazotype material, comprising a support carrying a light-sensitive layer containing a diazo compound of the general formula:



15 in which X is an anion, R<sub>1</sub> and R<sub>2</sub> are selected from the class consisting of chlorine and bromine atoms, and R<sub>3</sub> is selected from the class consisting of a cyclohexyl radical and methyl substituted cyclohexyl radicals.

2. One-component diazotype material according to claim 1, said support comprising a transparent sheet material coated with a film layer of a hydrophilic colloid formed by hydrolysis of an ester selected from the group consisting of cellulose and polyvinyl esters, which film layer contains said diazo compound together with a stabilizer selected from the group consisting of 1,3,6-naphthalene trisulphonic acid and water-soluble salts thereof.

3. One-component diazotype material according to claim 2, characterized in that the diazo compound is present in the film layer in the form of the zinc chloride double salt of said compound.

4. One-component diazotype material comprising a support carrying a light-sensitive layer containing a salt of 4 - N - methyl-N-cyclohexylamino-3,6-dibromo-diazo-benzene.

35 5. One-component diazotype material comprising a support carrying a light-sensitive layer containing a salt of 4 - N - methyl-N-cyclohexylamino-3,6-dichloro-diazo-benzene.

6. One-component diazotype material comprising a support carrying a light-sensitive layer containing a salt of 4-N-methyl-N-cyclohexylamino-3-chloro-6-bromo-diazo-benzene.

7. One-component diazotype material comprising a support carrying a light-sensitive layer containing a salt of 4-N-methyl-N-(methyl) cyclohexylamino-3,6-dichloro-diazo-benzene.

#### References Cited by the Examiner

##### UNITED STATES PATENTS

|           |         |                    |         |
|-----------|---------|--------------------|---------|
| 2,067,132 | 1/1937  | Schnitzpahn et al. | 260-141 |
| 2,405,523 | 8/1946  | Sease et al.       | 96-91 X |
| 2,548,845 | 4/1951  | Neumann            | 96-91   |
| 2,552,354 | 5/1951  | Von Glahn et al.   | 96-91   |
| 2,618,555 | 11/1952 | Reichel            | 96-91 X |
| 2,793,118 | 5/1957  | Sanders et al.     | 96-91   |
| 2,996,381 | 8/1961  | Oster et al.       | 96-91 X |

##### FOREIGN PATENTS

|    |         |         |                |
|----|---------|---------|----------------|
| 60 | 682,353 | 11/1952 | Great Britain. |
|----|---------|---------|----------------|

J. TRAVIS BROWN, Acting Primary Examiner.

NORMAN G. TORCHIN, ALEXANDER D. RICCI,  
Examiners.

R. L. STONE, R. SMITH, Assistant Examiners.